

Patented Feb. 15, 1927.

1,617,434

# UNITED STATES PATENT OFFICE.

KARL BINDER, OF STUTTGART, GERMANY.

## DEVELOPER FOR PHOTOGRAPHIC PLATES, FILMS, PAPERS, AND THE LIKE.

No Drawing. Application filed August 25, 1925, Serial No. 52,459, and in Great Britain July 14, 1925.

The present invention relates to a process for the manufacture of developers for photographic plates and the like.

The object of the invention is to provide a developer by which development can be carried out under any desired source of light, and particularly also in daylight.

The process consists essentially in adding an alkali to complex compounds of iron with polyvalent phenols such as potassium salt of tripyrocatechin ferric acid having the following chemical formula:



Suitable complex iron phenol compounds for the manufacture of daylight developers for photographic plates and the like are primarily alkali salts of tripyrocatechin-ferric acid. In addition to the said salts of tripyrocatechin-ferric acid the salts of dipyrrocatechin-ferric acid can also be used, as these violent salts can be easily converted by excess of alkali into the red salts of tripyrocatechin-ferric acid with the separation of ferric hydroxide. It has been observed that such complex compounds when dissolved in water have a powerful reducing action on photographic plates, films, papers, and the like coated with an emulsion sensitive to light, after the addition of the alkali, so that these solutions are admirably suitable for use as photographic developers. As the complex iron phenol compounds are only slightly dissociated in aqueous solution, they cannot be used as developers without the addition of an alkali, and only excess of alkali makes a good developer from them.

For the satisfactory development of photographic plates and the like even very dilute solutions in water of these complex compounds suffice when an alkali is present to secure good results. As under these circumstances only a small percentage of dissociated phenol comes into action, hydrolytically, these complex iron phenol compounds exert a surprising acceleration on the reaction during development. The intense red colour is, however, maintained during development, and ferric hydroxide is only separated in proportion as the phenol is consumed during development.

The red colour of the aqueous solutions of these complex iron phenol compounds makes them suitable for development under any source of light, also particularly by daylight. Under these circumstances it is mere-

ly necessary that the plates or the like be placed in the dark or in a red light in the developing bath.

The red colour of the solution prevents, firstly, as is well known, the chemically active rays from acting on the light sensitive emulsion. As soon as the light sensitive emulsion has been saturated with the developing solution, it has been rendered so thoroughly insensitive to light that the plates can be even repeatedly removed from the developer in any light, even daylight, in order to observe the progress of the development.

After development has been completed, the plates are rinsed with water and can be fixed in an acid fixing bath in any light, even in daylight, without any further precautions having to be taken. The plates are then washed.

### Example.

A developer of suitable composition is the following:—

2 grs. potassium salt of tripyrocatechin ferric acid, 198 ccm. distilled water, 15 ccm. 10% potassium hydroxide solution.

The plate to be developed, such as a Hauff ultra rapid plate, is placed after exposure in the said developer in a red light, after which the electric light can be switched on. After two or three minutes more the plate may be removed from the bath as many times as may be desired, both by a bright electric light and even in daylight, so as to observe the progress of the development. When the plate is developed, it is rinsed in water and fixed in an acid fixing bath of the following composition:—

25 grs. sodium thio-sulphate. 3 grs. sodium bi-sulphite, 72 ccm. distilled water.

Plates developed by the above method have the disadvantage of showing a light brown to a reddish brown colour after fixing. This is disadvantageous, as they require a slightly longer time in copying for the production of positives.

According to the present invention, this disadvantage is overcome by adding a water soluble sulphite to the daylight developer compounded according to the above process. This addition of the water soluble sulphite completely overcomes the above mentioned disadvantage. The emulsion of the plate is, however, normal in every respect, as it copies in normal time, for exam-

ple. The process may be illustrated by the following example:—

To prepare the developer 2 grs. potassium salt of tripyrocatechin ferric acid and 5 grs. 5 sodium sulphite (crystalline) are dissolved in 200 ccm. distilled water, and 10 ccm. of a 10% solution of potassium hydroxide are added.

The plates to be developed are placed in 10 the said developer in a red light, or in a dark room, or under an absolutely light-tight cloth after exposure, after which the electric light may be switched on at once, or daylight admitted. After two minutes 15 the plate may be removed from the developer repeatedly, both under a bright electric light, or even in daylight, in order to observe the progress of the development. After the plate has been developed, it is 20 rinsed off with water, and fixed in a fixing bath of the following composition:—

25 grs. sodium thio-sulphate, 5 grs. sodium bi-sulphite, 70 ccm. distilled water, and then washed.

25 I claim:—

1. A developer for photographic plates, films, papers, and the like, prepared by making an aqueous solution of a complex compound of iron with polyvalent phenols, 30 and adding an alkali thereto.

2. A developer for photographic plates, films, papers, and the like, prepared by making an aqueous solution of a complex compound of iron with polyvalent phenols, 35 and adding alkali in excess thereto.

3. A developer for photographic plates, films, papers, and the like, prepared by forming an aqueous solution of potassium salt of tripyrocatechin ferric acid, and adding an alkali thereto.

4. A developer for photographic plates, films, papers, and the like, prepared by forming an aqueous solution of potassium salt of tripyrocatechin ferric acid, and adding alkali in excess thereto.

5. A developer for photographic plates, films, papers, and the like, prepared by forming an aqueous solution of potassium salt of tripyrocatechin ferric acid, and adding potassium hydroxide solution thereto.

6. A developer for photographic plates, films, papers and the like, prepared by dis-

solving 2 grs. of potassium salt of tripyrocatechin ferric acid in 198 ccm. of distilled water, and adding 15 ccm. 10% solution of potassium hydroxide thereto.

7. A process of developing a photographic plate, film, paper, and the like, consisting in disposing the exposed negative in a developer prepared by dissolving 2 grs. of potassium salt of tripyrocatechin ferric acid in 198 ccm. of distilled water, and adding 15 ccm. 10% solution of potassium hydroxide thereto, rinsing the developed negative and fixing in a bath prepared by dissolving 25 grs. of sodium thio-sulphate and 3 grs. of sodium bisulphite in 72 ccm. of distilled water.

8. A developer for photographic plates, 70 films, papers, and the like, prepared by making an aqueous solution of a complex compound of iron with polyvalent phenols, and adding an alkali and a water soluble sulphite thereto for the purpose set forth.

9. A developer for photographic plates, films, papers, and the like prepared by making an aqueous solution of a complex compound of iron with polyvalent phenols, and adding alkali in excess and a water soluble sulphite thereto for the purpose set 80 forth.

10. A developer for photographic plates, films, papers, and the like, prepared by dissolving 2 grs. of potassium salt of tripyrocatechin ferric acid and 5 grs. of sodium 85 sulphite (crystalline) in 200 ccm. of distilled water and adding 10 ccm. of a 10% solution of potassium hydroxide thereto.

11. A process of developing a photographic plate, film, paper, or the like, consisting in disposing the exposed negative in a developer prepared by dissolving 2 grs. of potassium salt of tripyrocatechin ferric acid and 5 grs. of sodium sulphite (crystalline) in 200 ccm. of distilled water, and adding 10 ccm. of a 10% solution of potassium hydroxide thereto, rinsing the developed negative and fixing in a bath prepared by dissolving 25 grs. of sodium thio-sulphate and 5 grs. of sodium bi-sulphite in 70 ccm. 100 of distilled water.

In testimony whereof I affix my signature.

KARL BINDER.